

June 10, 1958

F. C. KELLEY

2,837,817

METHOD OF MAKING THIN METAL SHEETS

Filed Aug. 18, 1955



INVENTOR  
FLOYD C. KELLEY  
BY  
George Sipkin  
Levi Shulman  
ATTORNEYS

1

2,837,817

**METHOD OF MAKING THIN METAL SHEETS**

Floyd C. Kelley, Schenectady, N. Y., assignor, by mesne assignments, to the United States of America as represented by the Secretary of the Navy

Application August 18, 1955, Serial No. 529,368

7 Claims. (Cl. 29—424)

This invention relates to a method of preparing thin metal sheets and more particularly, for preparing formed parts of thin metal sheets such as molybdenum and tungsten.

In many situations, such as in miniature high-frequency power tubes, the mass of the cathode therein is an important factor because of the heat that must be dissipated. To cope with this factor, it is necessary to provide cathodes which have a very small mass. This can be accomplished by providing cathodes consisting of thin metal foils. However, it is particularly difficult to obtain thin foils of molybdenum or tungsten for cathode fabrication which are free from cracks and imperfection and it is also difficult to avoid further cracks or imperfections when the thin molybdenum or tungsten foil is shaped into a cathode cup.

Accordingly, it is the primary object of the present invention to provide a method of preparing sheets of metal foil which are free from cracks or imperfections.

It is a further object to provide a method of preparing sheets of molybdenum or tungsten having a thickness of 0.1 to 0.2 mil.

It is another object to provide a method of preparing cathode cups free from cracks and imperfections consisting of molybdenum or tungsten foil having a thickness of 0.1 to 0.2 mil.

In accordance with the present invention, there is provided a method of preparing thin molybdenum and tungsten foil which comprises the steps of cleaning one surface of a thin sheet of the molybdenum or tungsten and one surface of a thicker larger sheet of iron and then placing the clean surface of the molybdenum or tungsten sheet upon and within the periphery of the clean surface of the iron sheet. A sheet of stainless steel which is substantially equal in dimension to the iron sheet is placed upon the other surface of the molybdenum or tungsten sheet. A plurality of spaced spot welds between the iron and the stainless steel is made at the periphery to form a compact comprising the stainless steel, either molybdenum or tungsten and the iron. The compact is heated in an inert gas atmosphere to a temperature of about 800-900° C. and then the heated compact is rolled to reduce its total original thickness by about 35 to 45% and to firmly bond the molybdenum or tungsten to the iron. The reduced compact is further rolled to reduce its total original thickness by about 50-60% and to free the stainless steel from the compact leaving either a tungsten or molybdenum clad iron strip. The molybdenum clad iron strip may be further cold rolled to a chosen thickness after which the strip is annealed. The iron may be removed from the strip by dissolution or other chemical means to provide the thin molybdenum film which is free from cracks and imperfections. Iron is soluble in dilute sulphuric acid and hydrofluoric acid but molybdenum is insoluble in hydrofluoric and dilute sulphuric acids and the tungsten is insoluble in hydrofluoric acid so that a

2

choice of the proper acids may be made to dissolve the iron without affecting the molybdenum or tungsten.

Also in accordance with the present invention there is provided a method of preparing a cathode cup consisting either of a thin foil of either molybdenum or tungsten which comprises the steps of cleaning one surface of a clean sheet of molybdenum or tungsten having a thickness of from 1 to 4 mils and one surface of a larger sheet of iron having a thickness of  $\frac{1}{32}$  to  $\frac{3}{32}$  inch. The cleaned surface of the molybdenum or tungsten is placed upon the cleaned surface of the iron and within the periphery thereof. A sheet of stainless steel which is substantially equal in dimensions to the iron sheet is placed upon the other surface of the molybdenum sheet. A plurality of spot welds is made between the iron and stainless steel at the periphery to form a compact of the stainless steel, the molybdenum or tungsten and the iron. The compact is heated in a hydrogen atmosphere to a temperature of 800-900° C. and is rolled to reduce its total original thickness by about 35-45% and to firmly bond the molybdenum or tungsten to the iron. A further rolling is then made with said reduced compact to reduce its total original thickness by 50 to 60% and to free the stainless steel from the compact, leaving a molybdenum or tungsten clad iron strip. A further cold rolling of the molybdenum strip may be made to a total thickness of about 5 mils after which the strip is annealed. The strip is then shaped into a cup or cup-like structure and the iron is removed therefrom by chemical means, thereby providing a molybdenum cup-like structure having a thickness of 0.1 to 0.2 mil.

Other objects and many of the attendant advantages of this invention will be readily appreciated as the same becomes better understood by reference to the following detailed description.

The single figure illustrates a method in accordance with this invention.

Generally speaking, the process of the present invention is performed by placing a clean surface of a relatively thick slab of metal, preferably iron, in contact with a cleaned surface of a relatively thin slab of molybdenum or tungsten. The surfaces may be cleaned readily by the conventional method of grit blasting and subsequent wire brushing. A sheet of stainless steel which is not cleaned on either surface is placed upon the uncleansed surface of the molybdenum or tungsten. The resulting sandwich of stainless steel molybdenum or tungsten and iron is then spot welded around the periphery at intervals to form a compact. The molybdenum or tungsten sheet is intentionally made narrower in both dimensions than either the iron or the steel sheets which are substantially equal in thickness and dimensions so that the spot welds around the periphery are made between the iron and the steel.

The welded compact is then placed in a hydrogen furnace and heated to 800 to 900° C. A hydrogen furnace is selected since it furnishes an inert and a reducing atmosphere so that the tungsten or molybdenum, iron and steel are not subjected to any deleterious chemical action during the heating. Although a hydrogen atmosphere is preferable, it may be replaced by another inert gas atmosphere such as of nitrogen or one of the noble gases. The compact is then given a heavy reduction by passing it between the pressure rolls of a rolling mill. The first pass through the rolls may reduce the thickness of the compact by about 40% and will also cause the molybdenum or tungsten to be firmly bonded to the iron. A second pass reduces the original thickness about 50 to 60% and due to the elongation of the metal sheets and the cooling thereof, a rupture of the spot welds will take place and the stainless steel is freed from the compact leaving a molybdenum or tungsten clad iron strip. The

latter may be cold rolled to further reduce its thickness after which it is annealed. Such annealing may be any method well known in the art. After the annealing, it has been found that the molybdenum or tungsten is in substantially perfect condition and shows no cracks or imperfection.

The annealed molybdenum or iron strip may be treated to remove the iron therefrom to provide thin foil sheets of molybdenum and tungsten. Since iron is soluble in hydrofluoric acid and dilute sulphuric acid and since molybdenum is insoluble in both of these acids and tungsten is insoluble in hydrofluoric acid, in the case of the molybdenum clad iron strip, the iron may be removed by submersion in a solution of dilute sulphuric acid or hydrofluoric acid. In the case of the tungsten clad iron strip, the iron may be removed by submersion of the strip in a solution of hydrofluoric acid.

To make cathodes consisting of thin films of molybdenum or tungsten, either the molybdenum clad iron or tungsten clad iron strip is first shaped into the form of a cup before it is submerged into the iron dissolving acid. After the iron has been dissolved, there remains a cathode cup-like structure consisting either of molybdenum or tungsten. Since the molybdenum or tungsten provided on the strip is substantially free of cracks or imperfections and since the shaping operation of the strip into a cup-like structure does not cause cracks and imperfections, it is to be seen, that a cathode consisting of a substantially perfect foil of molybdenum or tungsten is provided by the present invention.

Typical quantities used to provide the present invention may be seen in the following example:

| Original Thickness of Iron, inch | Original Thickness of Molybdenum or Tungsten, mils | Original Thickness of Stainless Steel, inch |
|----------------------------------|----------------------------------------------------|---------------------------------------------|
| $\frac{1}{32}$ to $\frac{3}{32}$ | 1 to 4                                             | $\frac{1}{32}$ to $\frac{3}{32}$            |

First rolling: Reduction of 35 to 45% of original thickness.

Second rolling: Reduction of 50 to 60% of original thickness.

Third rolling: Reduction to a total thickness of about 5 mil. Dissolution of iron leaves a molybdenum or tungsten foil of 0.1 to 0.2 mil thickness.

In a precise embodiment of the present invention, the beginning materials were  $\frac{1}{16}$ " iron sheet, 2.5 mil molybdenum or tungsten sheet and  $\frac{1}{16}$ " stainless sheet, as described above. Of course, thicker sheets may be used to produce other final desired thicknesses.

Obviously many modifications and variations of the present invention are possible in the light of the above teachings. It is therefore to be understood that within the scope of the appended claims the invention may be practiced otherwise than as specifically described.

I claim:

1. A method of preparing a thin foil of a metal selected from the group consisting of molybdenum and tungsten which comprises the steps of cleaning one surface of a thin sheet of said metal and one surface of a thicker larger sheet of iron; placing the cleaned surface of said metal sheet against and within the periphery of the cleaned surface of said iron sheet; placing a sheet of uncleaned stainless steel which is substantially equal in dimensions to said iron sheet against the uncleaned surface of said metal sheet; making a plurality of spaced spot welds between said iron and said stainless steel at said periphery to form a compact comprising said stainless steel, said metal, and said iron; heating said compact in a noncorrosive atmosphere to a temperature of 800° C. to 900° C.; rolling said heat compact to reduce its total original thickness by about 35 to 45% and to

5 firmly bond said metal to said iron; further rolling said heated compact to further reduce its total original thickness by 50 to 60% and to free said stainless steel from said compact leaving a laminate of said metal and said iron; cold rolling said laminate to a chosen thickness; annealing said laminate; and then dissolving said iron away from said laminate whereby there is obtained a thin foil of said metal.

2. A method of preparing thin molybdenum foil which 10 comprises the steps of both cleaning one surface of a thin sheet of molybdenum and one surface of a thicker larger sheet of iron; placing the cleaned surface of said molybdenum sheet against and within the periphery of the cleaned surface of said iron sheet; placing a sheet of uncleaned stainless steel which is substantially equal in 15 dimensions to said iron sheet against the uncleaned surface of said molybdenum sheet; making a plurality of spaced spot welds between said iron and said stainless steel at said periphery to form a compact of said stainless steel, said molybdenum, and said iron; heating said compact in a hydrogen atmosphere to a temperature of 800 to 900° C.; rolling said heated compact to reduce its total original thickness by about 35% to 45% and to firmly bond said molybdenum to said iron; further 20 rolling said reduced heated compact to reduce its total original thickness by about 50% to 60% and to free said stainless steel from said compact leaving a molybdenum clad iron strip; cold rolling said molybdenum clad iron strip to a chosen thickness; annealing said strip; and then 25 removing the iron from said strip by dissolution thereof in a material selected from the group consisting of a hydrofluoric acid solution and a dilute sulphuric acid solution.

3. A method of preparing thin molybdenum foil which 30 comprises the steps of cleaning one surface of a thin sheet of molybdenum having a thickness of 1 to 4 mils and one surface of a larger sheet of iron having a thickness of  $\frac{1}{32}$  to  $\frac{3}{32}$  inch; placing the cleaned surface of said molybdenum sheet against and within the periphery of the cleaned surface of said iron sheet; placing a sheet of uncleaned stainless steel which is substantially equal in 35 dimensions to said iron sheet against the uncleaned surface of said molybdenum sheet; making a plurality of spaced spot welds between said iron and said stainless steel at said periphery to form a compact of said stainless steel, said molybdenum and said iron; heating said compact in a hydrogen atmosphere to a temperature of 800 to 900° C.; rolling said heated compact to reduce its total original thickness by about 35% to 45% and to firmly bond said molybdenum to said iron; further rolling said reduced heated compact to reduce its total original thickness by 40 50% to 60% and to free said stainless steel from said compact leaving a molybdenum clad iron strip; cold rolling said molybdenum clad iron strip to a total thickness of about 5 mils; annealing said strip; and then removing said iron therefrom by dissolution thereof in a material selected from the group consisting of a hydrofluoric acid solution and a dilute sulphuric acid solution 45 whereby there is provided a molybdenum foil having a thickness of 0.1 to 0.2 mil.

4. A method of preparing a cathode comprising a thin molybdenum foil which comprises the steps of cleaning one surface of a sheet of molybdenum having a thickness of 1 to 4 mils and one surface of a larger sheet of iron having a thickness of  $\frac{1}{32}$  to  $\frac{3}{32}$  inch; placing the cleaned surface of said molybdenum sheet against and within the periphery of the cleaned surface of said iron sheet; placing a sheet of uncleaned stainless steel which is substantially equal in dimensions to said iron sheet against the uncleaned surface of said molybdenum sheet; making a plurality of spaced spot welds between said iron and said stainless steel at said periphery to form a compact of said stainless steel, said molybdenum, and said iron; heating said compact in a hydrogen atmosphere to a temperature of 800 to 900° C.; rolling said heated 50 55 60 65 70 75 80 85 90 95

compact to reduce its total original thickness by about 35% to 45% and to firmly bond said molybdenum to said iron; further rolling said reduced heated compact to reduce its total original thickness to about 50 to 60% and to free said stainless steel from said compact leaving a molybdenum clad iron strip; cold rolling said molybdenum clad iron strip to a thickness of about 5 mils; annealing said strip; forming said annealed strip into a cup-like structure; and then removing the iron from said cup-like structure by dissolution thereof in material selected from the group consisting of a hydrofluoric acid solution and a dilute sulphuric acid solution whereby there is provided a cathode of cup-like structure consisting of a molybdenum foil of one of 0.1 to 0.2 mil thickness.

5. A method of preparing thin tungsten foil which comprises the steps of cleaning one surface of a thin sheet of tungsten and one surface of a thicker larger sheet of iron; placing the cleaned surface of said tungsten sheet against and within the periphery of the cleaned surface of said iron sheet; placing a sheet of uncleaned stainless steel which is substantially equal in dimensions to said iron sheet against the uncleared surface of said tungsten sheet; making a plurality of spaced spot welds between said iron and said stainless steel at said periphery to form a compact of said stainless steel, said tungsten, and said iron; heating said compact in a hydrogen atmosphere to a temperature of 800 to 900° C.; rolling said heated compact to reduce its total original thickness by about 35% to 45% and to firmly bond said tungsten to said iron; further rolling said reduced heated compact to reduce its total original thickness by about 50% to 60% and to free said stainless steel from said compact leaving a tungsten clad iron strip; further cold rolling said tungsten clad iron strip to a chosen thickness; annealing said strip and then removing said iron from said strip by dissolution thereof in hydrofluoric acid solution.

6. A method of preparing a thin tungsten foil which comprises the steps of cleaning one surface of a sheet of tungsten of 1 to 4 mils thickness and one surface of a larger sheet of iron having a thickness of  $\frac{1}{32}$  to  $\frac{3}{32}$  inch; placing the clean surface of said tungsten sheet against and within the periphery of the clean surface of said iron sheet; placing a sheet of uncleaned stainless steel which is substantially equal in area and thickness to said iron sheet against the uncleared surface of said tungsten sheet; making a plurality of spaced spot welds between said iron and said stainless steel at said periphery to form a compact of said stainless steel, said tungsten and said

40

45

50

55

60

65

70

75

80

85

90

95

100

iron; heating said compact in a hydrogen atmosphere to a temperature of 800 to 900° C. rolling said heated compact to reduce its total original thickness by about 35% to 45% and to firmly bond said tungsten to said iron; further rolling said reduced heated compact to reduce its total original thickness by 50% to 60% and to free said stainless steel from said compact leaving a tungsten clad iron strip; further cold rolling said tungsten clad iron strip to a thickness of about 5 mils; and then removing said iron from said strip by dissolution thereof in a solution of hydrofluoric acid whereby there is provided a tungsten foil having a thickness of 0.1 to 0.2 mil.

7. A method of preparing a cathode consisting of a thin tungsten foil which comprises the steps of cleaning one surface of a tungsten sheet having a thickness of 1 to 4 mils and one surface of a larger sheet of iron having a thickness of  $\frac{1}{32}$  to  $\frac{3}{32}$  inch; placing the clean surface of said tungsten sheet against and within the periphery of the clean surface of said iron sheet; placing a sheet of uncleanned stainless steel which is substantially equal in dimensions to said iron sheet against the uncleared surface of said tungsten sheet; making a plurality of spaced spot welds between said iron and said stainless steel at said periphery to form a compact of said stainless steel, said tungsten, and said iron; heating said compact in a hydrogen atmosphere to a temperature of 800 to 900° C.; rolling the heated compact to reduce said total original thickness by about 35% to 45% and to firmly bond said tungsten to said iron; further rolling said reduced heated compact to reduce its total original thickness by 50% to 60% and to free said stainless steel from said compact leaving a tungsten clad iron strip; further cold rolling said tungsten clad iron strip to a thickness of about 5 mils; annealing said strip; shaping said annealed strip to a cup-like structure; and removing said iron therefrom by the dissolution thereof in a hydrofluoric solution whereby there is provided a cup-like tungsten cathode consisting of a tungsten foil having a thickness of .1 to .2 mil.

#### References Cited in the file of this patent

#### UNITED STATES PATENTS

|           |          |               |
|-----------|----------|---------------|
| 827,696   | Lewis    | July 31, 1906 |
| 1,610,225 | Metcalf  | Dec. 7, 1926  |
| 1,886,615 | Johnson  | Nov. 8, 1932  |
| 1,956,818 | Acre     | May 1, 1934   |
| 1,981,915 | Hormel   | Nov. 27, 1934 |
| 2,423,810 | Goulding | July 8, 1947  |